

## UNITED STATES PATENT OFFICE

2,360,623

## LUBRICATING OIL COMPOSITION

Raphael Rosen, Elizabeth, N. J., assignor to  
Standard Oil Development Company, a corpora-  
tion of Delaware

No Drawing. Application March 1, 1941,  
Serial No. 381,388

6 Claims. (CL 252—44)

This invention relates to improvements in lubricating oil compositions. More particularly, it is concerned with hydrocarbon lubricating oils improved in stability by the addition of a quaternary phosphonium compound.

At the high temperatures of the order of 200° C., and higher, encountered in the operation of internal combustion engines, the instability of lubricating oils is associated with the susceptibility of these oils to undergo oxidation and thermal decomposition with resultant formation of corrosive substances and objectionable carbonaceous deposits on hot engine parts. As internal combustion engines are being designed and manufactured increasingly for higher power output, the requirements for greater stability in motor lubricants become steadily more stringent.

The main object of the present invention is to provide lubricating oil compositions of improved stability for satisfactory performance in the lubrication of internal combustion engines.

Advantageous effects on the stability of lubricating oils of various metallo-organic compounds containing a metallo-element selected from the second, third, and fifth groups of the periodic table of elements are described in my U. S. Patents No. 2,181,913, No. 2,181,914, and No. 2,181,915, all granted on December 6, 1939. My copending application, Serial No. 307,263, filed December 2, 1939, now issued as Patent No. 2,265,819 of December 9, 1941, of which the present application is a continuation-in-part, discloses organo-phosphorus compounds that are useful for stabilizing lubricating oils.

Among the different types of organo-phosphorus compounds considered for the purpose of improving lubricating oils are the phosphine derivatives of hydrogen phosphide,  $\text{PH}_3$ , in which organic radical substituents are directly linked to the phosphorus atom by carbon to phosphorus bonds. In these phosphines, organic radicals may be substituted for any or all of the three hydrogen atoms, giving the primary, secondary, and tertiary phosphines. Investigations have brought to light that while these phosphines, particularly the tertiary phosphines, have some value as antioxidants in stabilizing motor lubricants, they are surpassed in effectiveness by quaternary phosphonium compounds, which may be considered as additive compounds of the tertiary phosphines

and organic molecules containing a negative function, which usually has a halogen, sulfur, nitrogen, or an oxygen constituent.

The phosphonium stabilizing agents, with which the present invention is concerned, have compositions formulated as follows:

$[\text{R}_n\text{P}]_m\text{X}$

wherein R represents organic groups, i. e., chiefly hydrocarbon radicals selected from the type: alkyl, alkylene, cyclo-alkyl, aryl, alkaryl, and aralkyl; P represents a central quaternary phosphorus constituent in the molecule joined directly to carbon atoms of the R groups; and X represents a negative function such as a hydroxyl radical, a negative radical of an organic or inorganic acid, or the like. The subscript n denotes the number of R groups linked to the quaternary phosphorus constituent to satisfy exactly four valence bonds thereof. Of course, if the X group is polyvalent, the phosphonium radical  $[\text{R}_n\text{P}]$  must be combined in sufficient number, denoted by m, to satisfy the particular valence of X; e. g., if X is a sulfate radical, the generalized formula is  $[\text{R}_n\text{P}]_2\text{X}$ .

In the most readily procurable quaternary phosphonium compounds, each organic radical is monovalent, thus making the subscript n=4, but if the quaternary phosphorus constituent has a double bond linkage to a carbon atom, the subscript n will be less than 4, nevertheless, the compound still belongs to the quaternary phosphonium class of interest provided 4 valence bonds of the phosphorus are directly linked to carbon atoms.

It is to be understood that the R groups in the quaternary phosphonium compounds may be dissimilar and may contain substituent atoms, for example, halogen, nitrogen, oxygen, or sulfur, etc., or substituent groups, e. g. hydroxyl, alkoxy, carboxy, keto, amino, mercapto, etc. A number of compounds which illustrate these variations are: triphenyl ethyl phosphonium hydroxide and its salts, trimethyl cetyl phosphonium chloride, trimethyl allyl phosphonium naphthenate, phenyl benzyl dibutyl phosphonium dihydrogenphosphate, tricyclohexyl octadecyl phosphonium nitrate, tri (hydroxy-ethyl triamyl phosphonium) phosphite, tetrabenzyl phosphonium sulfate, tri-methyl chlorcetyl phosphonium acetate, triphenyl

octyl phosphonium hydroxide, and ethylene hexaethyl arsphosphonium bromide.

From extensive experience in using quaternary phosphonium and various metallo-organic compounds as lubricating oil additives, I have found that aromatic or aryl groups present among the R groups tend to improve the stability of these compounds and that alkyl groups among the R groups are favorable to the oil solubility of these compounds.

Since the quaternary phosphonium compounds are to be added to the lubricating oils for effecting the stabilization in very small concentrations of substantially less than 5% by weight, and generally as little as 0.01% to 1.0% by weight, they are as a class, adapted to be employed for the present purposes. The solubility of the quaternary phosphonium compounds can be modified by increasing the length and/or number of alkyl radicals, or a desired increase in concentration may be obtained with the aid of a solubilizing or dispersing agent. However, certain quaternary phosphonium compounds are pre-eminently suitable on account of their marked effectiveness and economical manufacture.

The preferred phosphonium compounds for stabilizing lubricating oils are the salts in which the quaternary phosphorus constituent is attached to 4 monovalent hydrocarbon radicals and the negative radical is an acid anion radical. These compounds are readily prepared and are particularly satisfactory in their stability and solubility characteristics.

At this point, it is desired to explain more fully the nature of the negative function as it exists in the quaternary phosphonium compounds. As a rule, this function is electronegative to both hydrogen and phosphorus and is present generally as an anion in combination with hydrogen in hydro acids, salts, or other ionizable compounds in which hydrogen acts as a cation. Some examples of these negative functions are the halide ions (e. g. Cl<sup>-</sup>, I<sup>-</sup>, Br<sup>-</sup>), the thiocyanate (SCN<sup>-</sup>), nitrate (NO<sub>3</sub><sup>-</sup>), sulfate (SO<sub>4</sub><sup>=</sup>), hydroxyl (OH<sup>-</sup>), phosphite (PO<sub>3</sub><sup>3-</sup>), bicarbonate (HCO<sub>3</sub><sup>-</sup>), acetate (CH<sub>3</sub>COO<sup>-</sup>), phenate, carbamate, and phenol sulfide radicals. It is recognized in the science of Chemistry that the atoms of elements and radicals are classifiable according to their degree of electronegativity to one another. The elements which are most non-metallic, e. g. the halogens, oxygen, sulfur, and nitrogen, are most electronegative, for atoms of such elements and radicals containing them have highly negative volt electron values as determined from their relative bond energies with other elements.

As previously mentioned, the tertiary phosphines, which are identified as the phosphines containing three carbon to phosphorus bonds or three monovalent hydrocarbon radicals attached to the trivalent phosphorus constituent, are capable of reacting with organic compounds containing a negative function to form quaternary phosphonium salts. These salts have been represented by various types of formulae, one of which is the following:



wherein X represents the negative function, e. g., the halogen atom in an alkyl halide, RX. This formula is used to represent the quaternary phosphonium salts as being molecular addition compounds.

The quaternary phosphonium salt formation reaction is represented, also, as follows:



in which, however, the negative function is regarded as not being attached directly to the phosphorus constituent, because the addition product of a tertiary phosphine molecule and another molecule containing a negative function behaves as if it consists of complex position ion [R<sub>4</sub>P]<sup>+</sup> associated with the anion function X<sup>-</sup>, giving these phosphonium compounds a peculiar ionic character which makes them differ very markedly from other organic compounds of phosphorus.

The tertiary phosphines are adapted for use as an initial material in producing the quaternary phosphonium salts, because they are capable of combining with the RX molecules, i. e. compounds such as alkyl halides and other organic compounds containing negative functions. The tertiary phosphines can be made by well-known methods from Grignard reagents or by other reactions, such as, dialkyl zinc compounds with PCl<sub>3</sub>. Typical examples of the tertiary phosphine compounds are triethyl phosphine (C<sub>2</sub>H<sub>5</sub>)<sub>3</sub>P, triphenyl phosphine (C<sub>6</sub>H<sub>5</sub>)<sub>3</sub>P, dibenzyl isoamyl phosphine



The quaternary phosphonium bases which are represented by [R<sub>4</sub>P]OH are also highly basic, being comparable in this respect to the quaternary ammonium bases and even to KOH. Accordingly, the quaternary phosphonium bases, which the phosphonium salts tend to form by hydrolysis, are readily neutralized by acids to the quaternary phosphonium salts. The quaternary phosphonium bases may be utilized in the present invention, and they first may be converted into salts, if so desired.

Quaternary phosphonium salts were prepared for use in the present invention by a classical procedure described in an article by Michaelis and Soden, Annalen, vol. 229, page 295 (1885). This procedure is exemplified in detail by the preparation of triphenyl ethyl phosphonium iodide as follows:

A 10 g. sample of triphenyl phosphine was placed in a flask with 20 cc. of ethyl iodide. The mixture was then refluxed on a water bath at 100° C. for a total of 10 hours. The product of the reaction was a yellow crystalline solid. Ether was added to the flask and the solid macerated therein. The solution was then filtered and the solid left on the filter was washed with more ether to remove impurities and then dried. This product, considered a crude product, weighed 16 g. making a 100% theoretical yield, and had a melting point of 163-166° C.

The crude product was dissolved in hot alcohol, filtered, and recrystallized from a mixture of alcohol and water to form colorless plate crystals. The weight of these crystals was 11.7 g. This refined product made a 73% theoretical yield and had a melting point corresponding closely to the melting point (146-165° C.) reported in the literature for triphenyl ethyl phosphonium iodide, (C<sub>6</sub>H<sub>5</sub>)<sub>3</sub>P(CH<sub>3</sub>)I.

To determine the relative merits of various compounds as stabilizing agents, in addition to service tests, the following analytical tests were conducted:

The cone test, which correlates with conditions and results obtained in internal combustion en-

gines in service, is used to quantitatively ascertain the amount of carbon-like material (in grams) deposited in two hours from a lubricating oil composition allowed to flow at a rate of 30 cc. per hour around a groove in a metal cone of standardized dimensions while the cone is held at a temperature of 250° C. The cones used are constructed of metals similar to those used in the construction of internal combustion engine parts.

This test indicates what effect the addition agent has in the formation of undesirable carbon-like deposits on hot engine parts.

Representative results from a series of runs on oil compositions are presented in the following example:

*Example*

A sample of refined lubricating oil, S. A. E. No. 50, used as a reference, or blank, was compared by the cone test with samples of the same oil to which were added, in one instance, 0.2% triphenyl arsine, in another, 0.2% of triphenyl phosphine, and in still another, between about 0.1 and 0.2% of triphenyl ethyl phosphonium iodide. Results of these tests are tabulated as follows:

| Lubricating oil composition                        | Cone test (deposit in grams) |
|----------------------------------------------------|------------------------------|
| Blank oil                                          | 0.50                         |
| Blank oil+0.2% triphenyl arsine                    | 0.36                         |
| Blank oil+0.2% triphenyl phosphine                 | 0.38                         |
| Blank oil+<0.2% triphenyl ethyl phosphonium iodide | 0.29                         |

From comparative data such as shown in the above table, it is noted that the quaternary phosphonium salt addition agent acts very efficiently in minimizing undesirable deposits on the hot metal surfaces.

To evaluate the oxidation inhibiting action of the quaternary phosphonium compounds in lubricating oil blends, the Oxygen Absorption Rate Test, which is a regularly employed standardized test for judging the ability of lubricants to resist oxidation under accelerated oxidation conditions, was used. This test is carried out by bubbling measured amounts of oxygen through the lubricating oil sample maintained at 200° C., the oxygen being continuously recycled. The amount of oxygen absorbed per 10 cc. of the oil sample is measured quantitatively at the end of each consecutive 15 minute period. The results are recorded as the number of cc. of oxygen absorbed per 10 cc. of oil during each 15 minute period. This test is carried out under conditions correlated to service conditions but with intensified action of pure oxygen intimately mixed with the oil. As a general rule, in this accelerated oxidation test the first two periods are the most crucial and indicative of the resistance of the oil to oxidation. In the first period there is an induction lag which makes the amount of oxygen absorbed relatively low, but in the second period the oxygen absorption reaches a peak or maximum after which the rate of absorption tends to decrease in a regular manner. Thus, it is ascertained from the data for the initial two or three periods how well the oil composition resists oxidation.

The samples of the same hydrocarbon lubricating oil (S. A. E. 50) used as a reference, or blank, were added small amounts of various inhibitors to be tested as anti-oxidants and results of the

oxidation tests on these samples are illustrated as follows:

| 10 | Sample tested                                      | Oxidation rate at 200° C.<br>cc. O <sub>2</sub> /10<br>cc. oil/15 min. |
|----|----------------------------------------------------|------------------------------------------------------------------------|
|    | Blank oil                                          | 103 213 107                                                            |
|    | Blank oil+0.2% triphenyl phosphine                 | 68 120 ...                                                             |
|    | Blank oil+<0.2% triphenyl ethyl phosphonium iodide | 20 36 28                                                               |

From the foregoing data on the oxidation rate, it can be observed that the quaternary phosphonium salt is more than three times as effective as the tertiary phosphine, from which it is derived, for retarding oxidation, and consequently considerably more effective for reducing deterioration of lubricating oils in this respect.

It is to be understood that one or more of the 20 quaternary phosphonium compounds, featured by this invention may be used to protect various types of hydrocarbon oils from deterioration by oxidation and thermal decomposition, particularly in motor lubricants, i. e. petroleum hydrocarbon oils having viscosities ranging upwardly from 60 Saybolt seconds at 100° F., i. e. upwardly in S. A. E. number beginning with an S. A. E. 10 lubricating oil. However, the oils to be improved may be more viscous, as in the case of semi-fluid 30 lubricants or greases, or less viscous. The oils to be used as a base in the lubricants may have high or low viscosity indices, may comprise fatty oils, natural or synthetic oils, bright stocks, or distillates, and may be finished by various refining processes, e. g. acid treating, absorptive clay refining, solvent extraction, selective precipitation, etc.

Other additives may also be incorporated in the lubricating oil compositions, as for example, 40 agents which aid in solubilizing and stabilizing the phosphonium compound, corrosion inhibitors, oiliness agents, oxidation inhibitors of other types, dyes, soaps, thickeners, viscosity index improvers, pour point depressors, solvents, sludge 45 dispersers, detergents, etc.

The present invention is not to be limited to any particular addition agent, nor to any theory as to the effect of these substances, nor to the particular amounts of the addition agents to be 50 used.

I claim:

1. A motor lubricating oil composition comprising a hydrocarbon lubricating oil and a small amount, sufficient to substantially stabilize said oil against oxidation, of a phosphonium compound having the type formula:

R<sub>n</sub>P<sub>1</sub>X

in which R represents hydrocarbon radicals and X is a halide anion.

2. A lubricant for rubbing metal surfaces comprising a hydrocarbon lubricating oil containing from 0.01% to 1% of triphenyl ethyl phosphonium iodide.

3. A lubricant for rubbing metal surfaces comprising a hydrocarbon lubricating oil and a small amount, sufficient to substantially stabilize said oil against oxidation, of a compound having the type formula:

[R<sub>n</sub>P]<sub>m</sub>X

70 wherein R<sub>n</sub> represents hydrocarbon radicals chosen to satisfy exactly four valence bonds of the quaternary phosphorus constituent and X represents an anion radical having a valence 75 number represented by m.

4. A lubricant for rubbing metal surfaces comprising a hydrocarbon lubricating oil containing a small amount, sufficient to substantially stabilize said oil against oxidation, of triphenyl ethyl phosphonium hydroxide.

5. A lubricant for rubbing metal surfaces comprising a hydrocarbon lubricating oil blended with a small amount, sufficient to substantially stabilize said oil against oxidation, of a quaternary phosphonium compound having the formula:



where  $R_1$ ,  $R_2$ ,  $R_3$ , and  $R_4$  are hydrocarbon radicals and  $X$  is an anion.

6. A lubricant for rubbing metal surfaces comprising a hydrocarbon lubricating oil blended with a small amount, sufficient to substantially stabilize said oil against oxidation, of a quaternary phosphonium compound having the formula:



where  $R_1$ ,  $R_2$ ,  $R_3$ , and  $R_4$  are hydrocarbon radicals and  $X$  is a salt-forming anion.

RAPHAEL ROSEN.